



US005213869A

**United States Patent** [19]**Magnani**[11] **Patent Number:** **5,213,869**[45] **Date of Patent:** **May 25, 1993**

[54] **CORRUGATED ROOFING SHEETS OF  
SYNTHETIC FIBER REINFORCED  
CEMENT, WITH A ROUGH SURFACE DUE  
TO THE PRESENCE OF GRANULAR  
MATERIAL**

[75] **Inventor:** **Sivio Magnani, Canneto Pavese, Italy**

[73] **Assignee:** **S.I.D.I. Societe Internationale de  
Developpements Industriels S.A.  
Holding, Luxembourg**

[21] **Appl. No.:** **555,605**

[22] **Filed:** **Jul. 23, 1990**

**Related U.S. Application Data**

[60] Division of Ser. No. 464,566, Jan. 16, 1990, Pat. No. 4,960,616, which is a continuation of Ser. No. 208,482, Jun. 20, 1988, abandoned.

**Foreign Application Priority Data**

Jul. 1, 1987 [IT] Italy ..... 21920/87[U]

[51] **Int. Cl.<sup>5</sup>** ..... **D06N 7/04; B32B 3/28**  
[52] **U.S. Cl.** ..... **428/143; 428/148;  
428/149; 428/150; 428/182; 428/196; 428/206;  
428/208; 428/210; 428/219; 428/325; 428/330;  
428/331; 428/332; 428/340; 428/402; 52/450;  
52/452; 52/537; 52/795**

[58] **Field of Search** ..... 428/141, 147, 148, 174,  
428/156, 182, 391, 394, 395, 425.5, 451, 454,  
143, 149, 196, 150, 219, 206, 208, 210, 325, 340,  
331, 330, 332, 402; 52/315, 450, 452, 454, 554,  
555, 558, 295, 659, 295, 782, 537, 795; 523/141,  
139, 204; 524/492, 493

**[56] References Cited****U.S. PATENT DOCUMENTS**

1,469,543 10/1923 Strachan et al. ..... 52/558  
1,868,803 7/1932 Overbury ..... 52/518  
1,890,023 12/1932 Schroder ..... 427/403  
2,307,734 1/1943 De Vault ..... 428/148  
2,798,822 7/1957 Carter ..... 427/186  
2,818,824 1/1958 Read et al. ..... 428/167  
3,376,629 4/1968 Baumann et al. ..... 428/138  
3,862,527 1/1975 Peterson ..... 52/94  
4,145,860 3/1979 Wotherspoon ..... 428/49  
4,241,107 12/1980 Mandish et al. ..... 427/140  
4,297,409 10/1981 Hannah ..... 428/294  
4,529,625 7/1985 Reidenbach et al. ..... 427/186

*Primary Examiner*—Donald J. Loney  
*Attorney, Agent, or Firm*—Parkhurst, Wendel & Rossi

**[57] ABSTRACT**

This invention relates to corrugated roofing sheets for building, made of a mixture of cement and inert materials, reinforced with synthetic fibers in fibrillated mesh form, characterized by having a rough outer surface due to the presence of surface granular material. The granular material is applied to the sheets during their finishing but before the cement has started to set, by simply strewing it over the sheet surface.

**5 Claims, No Drawings**

**CORRUGATED ROOFING SHEETS OF  
SYNTHETIC FIBER REINFORCED CEMENT,  
WITH A ROUGH SURFACE DUE TO THE  
PRESENCE OF GRANULAR MATERIAL**

This application is a Rule 60 divisional application of Ser. No. 07/464,566, filed Jan. 16, 1990, now U.S. Pat. No. 4,960,616, which in turn is Rule 62 continuation application of Ser. No. 07/208,482, filed Jun. 20, 1988, now abandoned.

**PRIOR ART**

Granular material is of known use in building components such as insulating sheets (French patent No. 2248384). Concrete components in the form of sheets with a rough surface and a vapour-impermeable film are also known (German patent No. 3022266), as are asbestos-cement sheets with granular material applied by pressing onto the surface of a cement layer superposed on the asbestos-cement (Japanese patent 53144926).

However, synthetic fiber reinforced cement sheets with a rough surface for roofing use in buildings are as yet unknown, notwithstanding the widespread requirement for such roofing sheets with non-slip characteristics which do not contain asbestos.

**SUMMARY OF THE INVENTION**

We have now found it possible to produce corrugated self supporting roofing sheets for buildings made of a cement and inert mixture reinforced with synthetic fibres in fibrillated mesh form, the sheets having a rough outer surface due to the presence of surface granular material applied by simple strewing.

Said sheets are produced in known continuously operating plants, by: preparing a layer of suitable thickness of a mix of cement and water with sand and other inert material, containing synthetic fibres in fibrillated mesh form, by either spraying the mix of cement and inert materials or allowing it to fall onto a felt or cloth band which advances continuously while supporting the fiber layer to be impregnated; strewing granular material over the surface of the layer before the cement starts to set; removing excess water from the layer by fixed or mobile suction boxes; cutting and corrugating the obtained sheets; and after the cement has set, brushing to remove from the surface those granules which have not been gripped by the cement.

The sheets of the present invention have functional and aesthetic characteristics which represent a considerable advance over components of the known art used for the same purpose, and their production cycle has advantageous aspects.

**DETAILED DESCRIPTION OF THE  
INVENTION**

This invention relates to corrugated or ribbed roofing sheets for buildings and the method for their production.

Said sheets are made of a cement and inert mixture reinforced with synthetic fibers which are characterized by possessing a rough outer surface due to the presence of surface granular material.

Said synthetic fibers are preferably polypropylene fibers in either fibrillated mesh form, and which have a much larger diameter than the asbestos fibers traditionally used in this field, namely between 15 and 120 mi-

crons compared with the diameters of asbestos fibers which are generally between 1 and 3 microns.

The granular material used for roughening the surface of the sheets according to the present invention is preferably grit produced from mineral substances such as limestone, marble, silica, granite etc. by grinding and sieving to a particle size of between 0.1 and 4 mm and preferably between 0.5 and 1.5 mm. The material can also consist of glass beads of the same size. The granular material is applied to the sheet surface in a quantity of between 200 and 1500 g/m<sup>2</sup> and preferably between 500 and 1000 g/m<sup>2</sup>.

The material is applied by distributing the granular material over the surface of the sheets during their finishing and before the cement has started to set. Thus, a layer of mix containing synthetic fibers is prepared to possess a thickness suitable for the sheet to be produced. The synthetic fibers are present to the extent of between 2.0 and 3.5% of the remaining solid material by weight.

The layer is prepared using a plant comprising a continuously advancing felt or cloth band on which the layer is deposited by free fall or spraying to engage the fibers which have been previously deposited. The layer surface consists essentially of cement, sand and any other additives, the synthetic fibers remaining distanced far apart and embedded in the mass since they are both thick and spread out.

As the sheet advances it is subjected to known finishing operations such as smoothing. At this point the granular material is strewn over the sheet surface, which consists essentially of wet cement and any inert additives, before the cement has started to set, after which the normal operations such as removing any excess water by suction boxes, cutting and corrugating, placing on steel forms and stacking are continued. Specifically, water removal is continued until the residual water content is between 25 and 32% and preferably between 27 and 29% of the weight.

As the cement sets, it grips the granules with which it comes into contact. When the cement is completely set, the sheet surface is brushed to remove those material granules which have not been gripped by the cement. The sheet corrugation profiles can be one of the known ranges corresponding, for example, to UNI 3949 177/6 or 146, ISO 691 or 692, or a different standard.

The sheets according to the invention have production, functional and aesthetic advantages compared with the known art. Their production process has, firstly, the advantage of comprising a simple and economical method of applying the granular material. A further advantage is the following: the corrugated sheets must be stacked with interposed plate steel forms between one sheet and the next in order to keep the shape of each sheet unaltered during setting of the cement. During this operation, if the synthetic fiber-reinforced sheets are not covered with granular material they will become scratched and marked at their points of contact with the plate steel forms, so that their final appearance will be deteriorated. This defect is inherent in components consisting of synthetic fiber-reinforced mixture of cement and inert materials because their surface consists essentially of cement. This does not, however, happen in the case of asbestos-cement since the asbestos reaches the surface to protect it from scratching. In the case of synthetic fiber-reinforced sheets without asbestos, the presence of the granular material makes the sheet surface insensitive to the action

of the plate steel forms, so that the sheets according to the invention preserve a perfect surface.

The sheets according to the invention also have the following advantages characteristics from a functional aspect:

when used directly as roofing sheets they obstruct the slippage of snow by virtue of the increased friction determined by the surface granular material;

when used as tile support sheets in which, when the roof is finished, their surface is not visible because it is covered by the tiles for which they act as a support, the increased friction between the sheet and tile prevents this latter slipping downwards. Furthermore, if the tiles are fixed by mortar, for example, to resist the under-thrust of the wind, the mortar adheres better to the rough surface of the sheet so that fixing is more secure;

in the case of only slightly inclined pitches, where the horizontal superimposed parts have to be sealed with mastic, the mastic is more easily retained by the rough surface and, consequently, the seal lasts longer since it better resists small to-and-fro movements which the roof undergoes due to temperature and humidity variations;

there is a reduced risk of slippage of the load distribution boards which maintenance personnel lay on the roof when walking on it, or of slippage of the actual personnel if walking directly on the roof;

in drilling the sheets to take the screws or nails used to fix the ridge tiles, the time loss due to easy lateral slippage of the drill bit on commencing drilling is avoided because, when the drill bit touches the surface to be drilled, the roughness produces an initial guide

sufficient to retain the bit in the required drilling position.

From aesthetic aspect the sheets have the following advantageous characteristics:

5 absence of undesirable reflection by virtue of a non-shiny surface;

better colour uniformity due to the absence of reflection;

regular and uniform ageing of the surface, the appearance of which always remains uniform with time because the film which forms with age adheres uniformly to every point by virtue of the considerable surface roughness.

I claim:

15 1. A corrugated self-supporting roofing sheet having a rough surface and consisting of a mixture of cement and sand reinforced with polypropylene fibers in fibrillated mesh form, said rough surface being due to granular material applied to the sheet surface, said granular material consisting of mineral substances ground and sieved to a particle size between 0.5 and 1.5 mm which are applied to said surface in a quantity between about 500 and about 1000 g/m<sup>2</sup> and said polypropylene fibers being present in an amount of between 2.0 and 3.5% by weight of the cement, sand and mineral substances.

20 2. The sheet of claim 1 wherein said granular material is limestone.

3. The sheet of claim 1 wherein said granular material is marble.

4. The sheet of claim 1 wherein said granular material is silica.

30 5. The sheet of claim 1 wherein said granular material is granite.

\* \* \* \* \*